

# UNITED STATES PATENT OFFICE.

JOHN HENRY HILL DUNCAN AND HARRY THEODORE BARNETT, OF  
LONDON, ENGLAND.

## INCANDESCENT STRUCTURE SUITABLE FOR LIGHTING.

SPECIFICATION forming part of Letters Patent No. 659,515, dated October 9, 1900.

Application filed October 26, 1899. Serial No. 734,878. (No model.)

*To all whom it may concern:*

Be it known that we, JOHN HENRY HILL DUNCAN, residing in the city of London, and HARRY THEODORE BARNETT, residing in Teddington, London, county of Surrey, England, subjects of the Queen of Great Britain and Ireland, have invented Improvements in Incandescent Structures Suitable for Lighting, of which the following is a specification.

10 This invention has reference to incandescent structures suitable for use as light-giving media when subjected to the action of heat—as, for example, when subjected to the action of non-luminous flames; and it has for 15 its objects, *inter alia*, to improve the color of the light furnished by such structures, to increase the strength of the structures, and to facilitate their manufacture, so that without departing from the more satisfactory 20 proportionate combinations of refractory substances incandescent structures can be produced whose color or tint of light and strength can be varied within reasonable limits.

Most incandescent structures of high efficiency as now prepared emit light other than 25 white—*i. e.*, a light possessing a preponderance of some one or more of the primary colors—as, for instance, the green-tinted-light-emitting Welsbach mantles and the orange-tinted-light-emitting mantles of the chrome class. According to this invention such 30 variously-tinted-light-emitting bodies are united or combined mechanically in one composite structure in such a manner that the selectively-emitted varying colors or tints of light 35 combine to produce an effect more pleasing to the eye or better suited to the purpose in view than heretofore. To this end we spin, double, knit, cable, interweave, overweave, 40 or otherwise mechanically connect or associate separate filaments, threads, cords, rods, fabrics, or other shaped bodies, hereinafter referred to as “filaments” or “threads,” containing or consisting of different proportionate 45 combinations of incandescent oxides which yield lights of different color or tint into one composite structure. By varying the number or size of the filaments containing each of the 50 said oxides or combinations of oxides used to form one thread or the number of threads of each employed to construct one composite

structure—it may be a mantle—or the positions of such differently-constituted members of such a thread, respectively, in relation to the position most favorable for radiating light 55 or for becoming heated to a maximum temperature we are enabled to produce incandescent bodies whose color or tint of light can be varied within comparatively-wide limits without departing from the more satisfactory 60 combinations of incandescent substances.

For ordinary purposes we sometimes prefer to combine filaments or threads of ceria-excited compounds or the like with filaments or threads of chrome compounds in order that 65 the approximately complementarily colored lights emitted by these different substances when rendered incandescent may unite to produce an illumination of more pleasant color than would be obtainable from either one of 70 them alone.

The filaments or threads of refractory-oxid-bearing material or of refractory oxid which are to be united according to this invention may be formed by the Welsbach or Knofer 75 processes or otherwise.

One or other of the kinds of filaments or threads constituting a composite incandescent structure according to this invention may be stronger than the remainder and so 80 render the whole mantle more durable or by reason of the said strength may allow a weaker substance—perhaps of higher light emissivity or possessing some other advantage—to be used in connection with it. In 85 some cases we adopt this compound construction of an incandescent structure, whereby it contains portions of differing constitution without particular reference to the color of light emitted for the reasons last above stated. 90

Incandescent mantles for use with gas-flames can be made according to this invention in various ways.

The following are examples of mantles giving a golden-white light. 95

First. Two lengths of cotton thread are soaked each in different solutions, one solution being such as to yield an incandescent body giving a light of greenish tint—for example, the well-known mixture or compound 100 of about ninety-nine per cent. thoria and one per cent. ceria—and the other solution being

such as yields an incandescent body containing fifty per cent. thoria, forty per cent. alumina, and ten per cent. chromic oxid. The soaked threads are dried and knitted, woven, 5 plaited, or otherwise intertwisted to form a mantle. The two threads may be knitted in such a manner that the mantle is composed of alternate rows of thoria-ceria and thoria-alumina chrome threads, or two or more rows 10 of either kind of thread may be used to one of the other. Another mode of making such mantles is to knit the fabric into a continuous length composed of alternately-arranged short sections of the different kinds of thread, 15 so that mantle lengths may be cut therefrom whose upper and lower portions are of different constitution. Mantles made by a weaving process may have the different kinds of threads equally distributed in the fabric, or 20 one kind of thread may be chiefly at the inner surface of the mantle, while the other kind is on the exterior surface of the mantle.

Second. Filaments containing two different mixtures of incandescent oxides are separately produced by the well-known Knofler or some similar process and the two kinds of filaments being doubled—*i. e.*, twisted—together to form a composite thread which is made into mantles in the usual way. One 25 kind of filament may contain thoria and ceria in or about the usual proportions and the other kind alumina chromic oxid and zirconia or thoria, a satisfactory prescription for the latter being thoria thirty-five per cent., chromic oxid five per cent., and alumina sixty 30 per cent., the alumina and thoria being conveniently added to the Knofler collodion in the form of nitrates of aluminium and thoriun and the chromic oxid as chromic acid, 35 and the two kinds of filaments being used in the proportion of twelve thoria-ceria filaments to three of the other kind.

Incandescent mantles made according to the foregoing examples give a light of golden-white color which does not become green in tint even when the mantles are well worn.

It will be obvious that more than two kinds of threads or filaments may be used and that different kinds of impregnated threads might 40 be doubled together to form one larger thread from which mantles can be made in the same way as from the composite Knofler thread and also that Knofler filaments of differing kind or composition need not necessarily be 45 united into one thread, but might be made into two or more different threads, which can be made into mantles in the manner hereinbefore described for the impregnated threads.

The burned-off alumina-containing threads 50 or filaments being stronger than the thoria-ceria threads or filaments their use tends to strengthen the mantle or that part of the mantle where they exist. If it is desired to 55 secure this strengthening effect without appreciably modifying the color of the light furnished by the thoria-ceria threads or filaments, the chromic oxid may be omitted from

the prescription. If desired, some other strengthening oxid or oxids, such as zirconia or silica, may be used in place of the alumina. 70

As hereinbefore stated, it is sometimes advantageous to cable—*i. e.*, to twist an external covering over a core—two or more kinds of filaments or threads together to constitute one larger thread, and in this case one kind of thread or filament may constitute the core, while another kind constitutes the lapping or covering. When the core of the cabled thread is of material which contracts more than the lapping or covering, the effect is to bow or 80 buckle the turns of lapping or covering material in such a manner that they are more readily permeated and heated by the flame in which the mantle is placed than would otherwise be the case. Sometimes the core may 85 contain a larger proportion of some constituent than it would be advisable to employ in threads or filaments which were to be wholly exposed. A durable thread of this kind may have a core of thoria-ceria in which the ceria 90 amounts to as much as or more than ten per cent., by weight, of the thoria present and a lapping or covering in which the thoria contains little or no ceria.

It is to be understood that we are aware 95 that it has heretofore been proposed to strengthen mantles by the addition to the mantle-body of supplementary threads or metallic wires applied to certain portions thereof; but such threads or wires are local only 100 in action, and owing to the variable contraction that takes place between the mantle-bodies and the supplementary threads or wires the latter tend to disintegrate the mantle-bodies rather than to strengthen them. 105

In incandescent bodies according to this invention the differently-constituted threads, filaments, or the like are united together in the process of manufacturing such bodies, as hereinbefore described, whereby a more 110 equally-distributed strengthening effect can be obtained without tending to disruption by reason of unequal contraction taking place between the different kinds of threads, filaments, or the like constituting the incandescent body. 115

What we claim is—

1. An incandescent structure suitable for lighting, comprising filaments or threads of different refractory substances arranged in 120 proximity to each other some of the filaments or threads being adapted to emit light of a different color to that emitted by the other filaments or threads substantially as described for the purpose specified. 125

2. An incandescent structure for lighting comprising mechanically-associated filaments or threads containing different substances or compounds, some of the filaments or threads being adapted to emit light of a different 130 color to that emitted by the other filaments or threads substantially as described for the purposes specified.

3. An incandescent structure comprising

mechanically-associated filaments or threads containing differing substances or compounds, one or some of which is or are adapted to complement the color of the light emitted by one or some of the others.

4. An incandescent structure comprising mechanically-associated filaments or threads containing differing substances or compounds, one or some of such filaments or threads being adapted to give a light of greenish tint and another or others a light of ruddy color.

5. An incandescent structure built up of interlaced filaments or threads one or some of which contain or contains a substance or compound adapted to complement the substance or compound contained in one or more of the other filaments or threads.

6. An incandescent structure built up of threads each of which consists of differing kinds of filaments adapted to complement each other as to the color of light emitted and as to strength as set forth.

7. An incandescent structure built up of interlaced filaments or threads some of which contain thoria and ceria and others chromic oxide and alumina, substantially as described.

8. An incandescent structure comprising mechanically-associated filaments or threads containing differing substances or compounds one or some of which filaments or threads are stronger than and support the other or others, substantially as described.

9. A composite incandescent structure for lighting composed of two different sets of interlaced filaments or threads each containing a different refractory oxid or oxides to the other substantially as herein described for the purposes set forth.

Signed at 39 Coleman street, London, E. C., 40 England, this 18th day of October, 1899.

JOHN HENRY HILL DUNCAN.

HARRY THEODORE BARNETT.

Witnesses:

C. H. WADMAN,  
H. E. SPINNEY.